

1

3,043,697

## PHOTOGRAPHIC GELATIN-N-VINYLLACTAM SILVER HALIDE EMULSIONS CONTAINING PHENOLIC ANTIFOGGANTS

Frederick Charles Forsgard, New Brunswick, N.J., assignor to E. I. du Pont de Nemours and Company, Wilmington, Del., a corporation of Delaware  
No Drawing. Filed Aug. 27, 1958, Ser. No. 757,460

4 Claims. (Cl. 96—109)

This invention relates to improved gelatin silver halide emulsions containing a poly-N-vinyllactam having 4 or 5 carbon atoms in the heterocyclic ring and fog inhibiting amounts of a monohydric or dihydric phenol anti-fogging agent.

It has been found that when a substantial percentage of the gelatin present in aqueous photographic emulsions is replaced by a poly-N-vinyllactam of the above class the resulting photographic silver halide emulsions have markedly increased covering power. The maximum density, contrast and effective speed of these poly-N-vinyl-lactam modified gelatin emulsions is also improved. However, applicant has found that such modified gelatin emulsions show a greater tendency to fog under conditions of storage, particularly conditions of high temperature and high relative humidity such as is encountered in storage in the tropical regions of the earth.

An object of this invention is to provide a simple and effective process for reducing the fogging tendencies of gelatino silver halide photographic emulsions containing poly-N-vinyllactams having 4 to 5 carbon atoms in the heterocyclic ring. Another object is to provide such a process which uses available chemical compounds of simple structure. Yet another object is to provide such a process which involves simple mixing procedures. A further object is to provide photographic gelatino silver halide emulsions containing substantial amounts of poly-N-vinyllactams which have enhanced covering power and contrast characteristics and which do not evidence any substantial increase in fog or loss in speed under high temperature or humidity conditions during storage. Still further objects will be apparent from the following description of the invention.

It has now been discovered, in accordance with the present invention, that photographic gelatino silver halide emulsions containing 8 to 50% by weight based on the weight of total solids in the emulsion of a water-soluble N-vinyllactam polymer containing 4 to 5 carbon atoms in the heterocyclic ring having an average molecular weight of at least 20,000 up to 200,000 or more, enhanced covering power and contrast and being stabilized against fog can be made by admixing with the emulsion small amounts from 5 to 50 millimoles per mole of silver halide of a phenol antifogging agent.

The mono or dihydric phenol antifogging agents can be added to the aqueous gelatin/poly-N-vinyllactam silver halide emulsion or dispersion at any time but are preferably added to the aqueous molten or liquefied emulsion after it has been brought to its maximum sensitivity and just prior to coating onto a suitable support to form a photographic film, plate or paper. Other emulsion adjuvants e.g., sulfur sensitizers, hardeners and optical sensitizing agents can be added to the emulsions previously, simultaneously or subsequent to the addition of the phenol.

The phenol antifogging agents can be added from ethanol solution (e.g., 2% by weight) or in some cases can be added to the emulsions described above. A particularly useful class of monohydric phenols wherein the

2

hydroxyl group is attached to a benzene nucleus can contain a hydrocarbon substituent in the para-position to the hydroxyl group and have one, two or three of the remaining nuclear hydrogen atoms substituted by hydrocarbon groups. Among the hydrocarbon substituents which may be present in the para-position and in the other positions of the benzene ring are alkyl radicals of 1 to 18 carbon atoms, e.g., methyl, ethyl, n-propyl, isopropyl, t-butyl, sec-amyl, t-amyl, t-octyl, n-nonyl and n-dodecyl; aryl, e.g., phenyl, naphthyl and biphenyl; aralkyl, e.g., benzyl,  $\alpha$ -cumyl and naphthylmethyl, and cycloalkyl, e.g., cyclopentyl and cyclohexyl. Specific compounds of this type are described below and in assignee's Smith application Serial No. 656,195, filed May 1, 1957, U.S. Patent 2,955,037, Oct. 4, 1960.

Another and related class of phenol antifogging agents which are particularly useful in accordance with the present invention are the hydrocarbon-substituted mono-nuclear monohydric phenols of at least 10 carbons wherein the hydrocarbon substituent is in one of the positions ortho- and meta- to the hydroxyl group and the other positions of the benzene ring are unsubstituted. These phenols have the general formula:



25

30

wherein one of the radicals R and R' is hydrogen and the other is a hydrocarbon radical of at least 4 carbon atoms. The hydrocarbon radicals may be alkyl, cycloalkyl, aryl and aralkyl. The alkyl radicals may contain 4 to 12 or more carbon atoms and suitable alkyl radicals are t-butyl, sec-amyl, t-amyl and t-octyl, n-nonyl and n-dodecyl. Suitable cycloalkyl radicals are cyclopentyl and cyclohexyl. Useful aryl radicals include phenyl, naphthyl and biphenyl. Suitable aralkyl radicals include benzyl,  $\alpha$ -cumyl and naphthylmethyl. Suitable specific compounds of this type are described below and in assignee's copending Smith application Serial No. 656,181, filed May 1, 1957 abandoned but refiled as continuation-in-part U.S. application Ser. No. 859,108, Patent 2,965,487, Dec. 20, 1960.

Yet another class of suitable phenols having anti-fogging properties are the bisphenols of the general formula

50

55



where Q is a direct carbon-to-carbon linkage —S—, —O—,  $(-\text{CH}_2-)_n$  where n is 1 to 10, or

60



where each of R and R<sub>1</sub> is an alkyl radical of 1 to 18 carbon atoms, R' and R'' are the same or different and are hydrogen, alkyl of 1 to 18 carbon atoms, cycloalkyl, or aryl, and the hydroxyl groups preferably are in the o- or p-position to the radical —Q—.

In the above formula suitable alkyl radicals include methyl, ethyl, propyl, isopropyl, n-butyl, t-butyl, pentyl, n-hexyl, n-octyl and t-octyl. Useful aryl radicals include phenyl and naphthyl, and suitable cycloalkyl radicals are cyclopentyl and cyclohexyl.

Many of the bis-type phenols useful in the invention are commercially available and others can be made in like manner by any of the known prior art procedures including those described in British specification 621,004 and 622,977; U.S. Patent 2,506,486 and those described in J. Am. Chem. Soc. vol. 54, 4325-34 (1932) and vol. 59, 1114 (1937) and Proc. Roy. Soc. vol. 129B, 528-538 (1940). The use of such bis-type phenols in gelatino-silver halide emulsions is described in Smith U.S. Patent 2,955,038, Oct. 4, 1960.

The invention is not limited to any particular type of light-sensitive silver halide as it is useful with silver chloride, silver bromide, silver iodobromide, silver chlorobromide, silver iodide, etc., emulsions and mixed emulsions of these types. It is particularly efficacious in silver iodobromide emulsions containing about 2 mole percent iodide and the rest bromide. These emulsions may be sensitized by means of chemical sensitizing agents, e.g. noble metal sensitizers, e.g., gold salts, e.g., chlorauric acid and auric trichloride, may be present in association with sulfur sensitizers, e.g., sodium sulfite, thiosinamine, allylthiourea, sodium thiosulfate, allyl thiocarbamate, alkali metal thiocyanates and sodium sulfide, these sensitizers to be used in amounts up to 0.005% based on the weight of the silver halide. Moreover, the silver halide emulsions may contain one or more optical sensitizing agents, e.g., cyanine, carbocyanine, merocyanine, pseudocyanine, cyazine, etc., dyes.

In general, the finished emulsions will contain on a dry basis, by weight, 8 to 50% poly-N-vinylactam, 30 to 70% silver halide and 10 to 60% gelatin and 5 to 50 millimoles per mole of silver halide of the phenol anti-fogging agent.

The invention will now be illustrated in and by the following examples wherein the parts and percentages stated are by weight unless otherwise indicated. The preparation of the emulsions, coating and storage of the photographic elements were carried out in the absence of actinic radiations. Also the covering powers shown in the following tables of the examples have been determined on the basis of 40 mg. of developed silver per square decimeter.

#### Example 1

A high speed gelatino-silver iodobromide (about 2 mole percent iodide, 98% bromide) was digested with an organic sulphur sensitizing compound and gold chloride. After digestion the emulsion was divided into three parts. One part was treated with 45.5 grams of poly-N-vinyl-2-pyrrolidone having an average molecular weight of approximately 45,000 per mole of silver halide. To a second part of emulsion were added 45.5 grams of poly-N-vinyl-2-pyrrolidone and 18 millimoles of resorcinol per mole of silver halide. The third part containing neither of the above additions was used as a control. The emulsions were coated on cellulose acetate film base and were exposed to X-rays in the presence of an intensifying screen at two different intensity levels through an aluminum  $\sqrt{2}$  step wedge. The exposure of greater intensity has been designated as No. 2 and that of lower intensity and longer time as No. 1.

The coatings were developed for 5 minutes in a developer of the following composition:

|                                     |       |      |
|-------------------------------------|-------|------|
| N-methyl-p-aminophenol hydrosulfate | grams | 3    |
| Anhydrous sodium sulfite            | do    | 50   |
| Hydroquinone                        | do    | 9    |
| Anhydrous potassium carbonate       | do    | 50   |
| Potassium bromide                   | do    | 4.5  |
| Water to make                       | ml    | 1000 |

The coatings were tested fresh, after one month of room aging, and after one week at 120° F. and 65% relative humidity (R.H.). The aged materials were exposed and developed as above. Results of tests for speed, gamma and fog before and after the storage treatment of each of the samples are given below. Speed is given in terms of a reciprocal of exposure at a density of 0.7.

#### FRESH RESULTS

| Compound                   | Amount per mole             | No. 2 exposure |       | No. 1 exposure |       | Fog | Covering power |
|----------------------------|-----------------------------|----------------|-------|----------------|-------|-----|----------------|
|                            |                             | Speed          | Gamma | Speed          | Gamma |     |                |
| Control                    | None                        | 830            | 2.70  | 450            | 2.31  | .05 | 30.8           |
| Polyvinyl pyrrolidone (I.) | 45.5 g.                     | 800            | 4.64  | 460            | 3.77  | .07 | 39.5           |
| I plus resorcinol          | 45.5 g. (I), 18 millimoles. | 800            | 4.31  | 460            | 3.52  | .06 | 39.0           |

#### ONE MONTH ROOM AGING

|                   | No. 2 exposure |       | No. 1 exposure |       | Fog |
|-------------------|----------------|-------|----------------|-------|-----|
|                   | Speed          | Gamma | Speed          | Gamma |     |
| Control           | 830            | 2.59  | 460            | 2.25  | .09 |
| I                 | 880            | 3.86  | 510            | 3.32  | .17 |
| I plus resorcinol | 840            | 3.89  | 550            | 3.21  | .10 |

#### ONE WEEK AT 120° F. AND 65% R.H.

|                          |  | Fog  |
|--------------------------|--|------|
| Control                  |  | .22  |
| I                        |  | 1.42 |
| I plus phenolic compound |  | .54  |

#### Example 2

The gelatino-silver iodobromide emulsion of Example 1 digested with sulphur and gold sensitizing compounds was divided into three parts. One part was treated with 45.5 grams of the poly-N-vinyl-2-pyrrolidone described in Example 1 per mole of silver halide. To a second part there were added 45.5 grams of the polymer and 20 millimoles of p-alpha-cumylphenol per mole of silver halide. Neither of these additions was made to a third part of the emulsion.

Coating, exposure, development and aging were carried out as in Example 1.

#### FRESH RESULTS

| Compound | Amount per mole             | No. 2 exposure |       | No. 1 exposure |       | Fog | Covering power |
|----------|-----------------------------|----------------|-------|----------------|-------|-----|----------------|
|          |                             | Speed          | Gamma | Speed          | Gamma |     |                |
| Control  | None                        | 780            | 3.51  | 360            | 2.64  | .06 | 32.5           |
| I        | 45.5 g.                     | 830            | 4.28  | 410            | 3.42  | .10 | 40.0           |
| I+phenol | 45.5 g. (I), 20 millimoles. | 830            | 3.84  | 460            | 3.16  | .08 | 39.5           |

#### ONE MONTH ROOM AGING

|                   | No. 2 exposure |       | No. 1 exposure |       | Fog |
|-------------------|----------------|-------|----------------|-------|-----|
|                   | Speed          | Gamma | Speed          | Gamma |     |
| Control           | 710            | 3.35  | 360            | 2.76  | .05 |
| I                 | 840            | 3.73  | 500            | 3.26  | .19 |
| I+phenol compound | 780            | 3.57  | 470            | 3.00  | .08 |

ONE WEEK AT 120° F. AND 65% R.H.

|          |  |  |  | Fog |
|----------|--|--|--|-----|
| Control  |  |  |  | .05 |
| I        |  |  |  | .76 |
| I+phenol |  |  |  | .38 |

## Example 3

The gelatino-silver iodobromide emulsion of Example 1 digested with sulphur and gold sensitizing compounds was divided into three parts. One part was treated with 45.5 grams of the poly-N-vinyl-2-pyrrolidone described in Example 1 per mole of silver halide. To a second part of the emulsion there were added 45.5 grams of the polymer, 24 millimoles of 2-benzyl-4-methyl-6-t-butyl-phenol and 6 millimoles of tri-t-butyl-p-phenylphenol per mole of silver halide. None of these additions was made to a third part of the emulsion.

Coating, exposure, development and aging were carried out as in Example 1.

## FRESH RESULTS

| Compound | Amount per mole             | No. 2 exposure |       | No. 1 exposure |       | Fog | Covering power |
|----------|-----------------------------|----------------|-------|----------------|-------|-----|----------------|
|          |                             | Speed          | Gamma | Speed          | Gamma |     |                |
| Control  | None                        | 830            | 2.79  | 450            | 2.31  | .05 | 30.8           |
| I        | 45.5 g.                     | 800            | 4.64  | 460            | 3.77  | .07 | 39.5           |
| I+phenol | 45.5 g. (I), 30 millimoles. | 800            | 4.16  | 460            | 3.26  | .06 | 39.0           |

## ONE MONTH ROOM AGING

|          | No. 2 exposure |       | No. 1 exposure |       | Fog |
|----------|----------------|-------|----------------|-------|-----|
|          | Speed          | Gamma | Speed          | Gamma |     |
| Control  | 830            | 2.59  | 830            | 2.59  | .09 |
| I        | 880            | 3.86  | 880            | 3.86  | .17 |
| I+phenol | 800            | 4.26  | 800            | 4.26  | .11 |

## Example 4

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion there were added 45.5 grams of the polymer and 9 millimoles of p-t-butylphenol per mole of silver halide. Neither of these additions was made to a third part of the emulsion.

Coating, exposure, development and aging were carried out as in Example 1.

## FRESH RESULTS

| Compound | Amount per mole            | No. 2 exposure |       | No. 1 exposure |       | Fog | Covering power |
|----------|----------------------------|----------------|-------|----------------|-------|-----|----------------|
|          |                            | Speed          | Gamma | Speed          | Gamma |     |                |
| Control  | None                       | 830            | 2.79  | 450            | 2.31  | .05 | 30.8           |
| I        | 45.5 g.                    | 800            | 4.64  | 460            | 3.77  | .07 | 39.5           |
| I+phenol | 45.5 g. (I), 9 millimoles. | 850            | 4.21  | 476            | 3.16  | .07 | 40.5           |

## ONE MONTH ROOM AGING

|          | No. 2 exposure |       | No. 1 exposure |       | Fog |
|----------|----------------|-------|----------------|-------|-----|
|          | Speed          | Gamma | Speed          | Gamma |     |
| Control  | 830            | 2.59  | 460            | 2.25  | .09 |
| I        | 880            | 3.86  | 510            | 3.32  | .17 |
| I+phenol | 910            | 3.47  | 490            | 2.94  | .12 |

ONE WEEK AT 120° F. AND 65% R.H.

| 5        |         |   |          |  | Fog  |
|----------|---------|---|----------|--|------|
|          | Control | I | I+phenol |  |      |
| Control  |         |   |          |  | .22  |
| I        |         |   |          |  | 1.42 |
| I+phenol |         |   |          |  | 1.04 |

## Example 5

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion there were added 45.5 grams of the polymer and 20 millimoles of 3,4 dimethyl phenol per mole of silver halide. Neither of these additions was made to a third part of the emulsion.

Coating, exposure, development and aging were carried out as in Example 1.

## FRESH RESULTS

| 25       | Compound                    | Amount per mole | No. 2 exposure |       | No. 1 exposure |       | Fog  | Covering power |
|----------|-----------------------------|-----------------|----------------|-------|----------------|-------|------|----------------|
|          |                             |                 | Speed          | Gamma | Speed          | Gamma |      |                |
| Control  | None                        | 780             | 3.51           | 360   | 2.64           | .06   | 29.0 |                |
| I        | 45.5 g.                     | 830             | 4.20           | 410   | 3.42           | .10   | 37.0 |                |
| I+phenol | 45.5 g. (I), 20 millimoles. | 880             | 4.16           | 460   | 3.45           | .10   | 36.5 |                |

## ONE MONTH ROOM AGING

| 35       |  | No. 2 exposure |       | No. 1 exposure |       | Fog |
|----------|--|----------------|-------|----------------|-------|-----|
|          |  | Speed          | Gamma | Speed          | Gamma |     |
| Control  |  | 710            | 3.35  | 360            | 2.70  | .05 |
| I        |  | 840            | 3.73  | 500            | 3.26  | .19 |
| I+phenol |  | 800            | 3.84  | 500            | 3.09  | .10 |

## ONE WEEK AT 120° F. AND 65% R.H.

| 45       |         |   |          |  | Fog |
|----------|---------|---|----------|--|-----|
|          | Control | I | I+phenol |  |     |
| Control  |         |   |          |  | .05 |
| I        |         |   |          |  | .76 |
| I+phenol |         |   |          |  | .66 |

## Example 6

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion there were added 45.5 grams of the polymer and 20 millimoles of o-phenylphenol per mole of silver halide. Neither of these additions was made to a third part of the emulsion.

Coating, exposure, development and aging were carried out as in Example 1.

## FRESH RESULTS

| 65       | Compound                    | Amount per mole | No. 2 exposure |       | No. 1 exposure |       | Fog  | Covering power |
|----------|-----------------------------|-----------------|----------------|-------|----------------|-------|------|----------------|
|          |                             |                 | Speed          | Gamma | Speed          | Gamma |      |                |
| Control  | None                        | 780             | 3.51           | 360   | 2.64           | .06   | 29.0 |                |
| I        | 45.5 g.                     | 830             | 4.28           | 410   | 3.42           | .10   | 37.0 |                |
| I+phenol | 45.5 g. (I), 20 millimoles. | 820             | 3.86           | 450   | 3.28           | .08   | 38.0 |                |

## ONE MONTH ROOM AGING

|               | No. 2 exposure |       | No. 1 exposure |       | Fog |
|---------------|----------------|-------|----------------|-------|-----|
|               | Speed          | Gamma | Speed          | Gamma |     |
| Control.....  | 710            | 3.35  | 360            | 2.70  | .05 |
| I.....        | 840            | 3.73  | 500            | 3.26  | .19 |
| I+phenol..... | 770            | 3.66  | 530            | 3.19  | .09 |

10

## ONE WEEK AT 120° F. AND 65% R.H.

|                    | Fog   |       |       |       |
|--------------------|-------|-------|-------|-------|
|                    | Speed | Gamma | Speed | Gamma |
| Control.....       |       |       |       | .05   |
| I.....             |       |       |       | .76   |
| I plus phenol..... |       |       |       | .38   |

## Example 7

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion were added 45.5 grams of the polymer and 10 millimoles of 4,4' isopropylidene-bisphenol per mole of silver halide. Neither of these additions was made to a third part of the emulsion.

Coating, exposure, development and aging were carried out as in Example 1.

## FRESH RESULTS

| Compound           | Amount per mole            | No. 2 exposure |       | No. 1 exposure |       | Fog | Covering power |
|--------------------|----------------------------|----------------|-------|----------------|-------|-----|----------------|
|                    |                            | Speed          | Gamma | Speed          | Gamma |     |                |
| Control.....       | None.....                  | 780            | 3.51  | 360            | 2.64  | .06 | 29.0           |
| I.....             | 45.5 g. (I)                | 830            | 4.28  | 410            | 3.42  | .10 | 37.0           |
| I plus phenol..... | 45.5 g. (I), 10 millimoles | 830            | 4.01  | 440            | 3.09  | .08 | 38.0           |

40

## ONE MONTH ROOM AGING

|                    | No. 2 exposure |       | No. 1 exposure |       | Fog |
|--------------------|----------------|-------|----------------|-------|-----|
|                    | Speed          | Gamma | Speed          | Gamma |     |
| Control.....       | 710            | 3.35  | 360            | 2.70  | .05 |
| I.....             | 840            | 3.73  | 500            | 3.26  | .19 |
| I plus phenol..... | 780            | 3.79  | 530            | 3.20  | .10 |

50

## ONE WEEK AT 120° F. AND 65% R.H.

|                    | Fog   |       |       |       |
|--------------------|-------|-------|-------|-------|
|                    | Speed | Gamma | Speed | Gamma |
| Control.....       |       |       |       | .05   |
| I.....             |       |       |       | .76   |
| I plus phenol..... |       |       |       | .32   |

55

## Example 8

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion there were added 45.5 grams of the polymer and 20 millimoles of p-benzylphenol per mole of silver halide. Neither of these additions was made to a third part of the emulsion.

Coating, exposure, development and aging were carried out as in Example 1.

65

## ONE WEEK AT 120° F. AND 65% R.H.

70

75

75

## 8 FRESH RESULTS

| Compound           | Amount per mole            | No. 2 exposure |       | No. 1 exposure |       | Fog | Covering power |
|--------------------|----------------------------|----------------|-------|----------------|-------|-----|----------------|
|                    |                            | Speed          | Gamma | Speed          | Gamma |     |                |
| Control.....       | None.....                  | 800            | 3.11  | 390            | 2.49  | .06 | 25.5           |
| I.....             | 45.5 g. (I)                | 850            | 4.00  | 450            | 3.28  | .10 | 35.4           |
| I plus phenol..... | 45.5 g. (I), 20 millimoles | 850            | 3.85  | 490            | 3.03  | .08 | 36.1           |

## ONE MONTH ROOM AGING

|                    | No. 2 exposure |       | No. 1 exposure |       | Fog |
|--------------------|----------------|-------|----------------|-------|-----|
|                    | Speed          | Gamma | Speed          | Gamma |     |
| Control.....       | 750            | 3.22  | 390            | 2.45  | .05 |
| I.....             | 800            | 3.55  | 440            | 2.93  | .14 |
| I plus phenol..... | 770            | 3.47  | 440            | 2.70  | .08 |

## ONE WEEK AT 120° F. AND 65% R.H.

|                    | Fog   |       |       |       |
|--------------------|-------|-------|-------|-------|
|                    | Speed | Gamma | Speed | Gamma |
| Control.....       |       |       |       | .26   |
| I.....             |       |       |       | .95   |
| I plus phenol..... |       |       |       | .62   |

## Example 9

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion there were added 45.5 grams of the polymer and 10 millimoles of m-t-butylphenol per mole of silver halide. Neither of these additions was made to a third part of the emulsion.

Coating, exposure, development and aging were carried out as in Example 1.

## FRESH RESULTS

| Compound           | Amount per mole            | No. 2 exposure |       | No. 1 exposure |       | Fog | Covering power |
|--------------------|----------------------------|----------------|-------|----------------|-------|-----|----------------|
|                    |                            | Speed          | Gamma | Speed          | Gamma |     |                |
| Control.....       | None.....                  | 800            | 3.11  | 390            | 2.49  | .06 | 25.5           |
| I.....             | 45.5 g. (I)                | 850            | 4.00  | 450            | 3.28  | .10 | 35.4           |
| I plus phenol..... | 45.5 g. (I), 10 millimoles | 850            | 3.91  | 460            | 3.17  | .09 | 34.8           |

## ONE MONTH ROOM AGING

|                    | No. 2 exposure |       | No. 1 exposure |       | Fog |
|--------------------|----------------|-------|----------------|-------|-----|
|                    | Speed          | Gamma | Speed          | Gamma |     |
| Control.....       | 750            | 3.22  | 390            | 2.45  | .05 |
| I.....             | 800            | 3.55  | 440            | 2.93  | .14 |
| I plus phenol..... | 830            | 3.84  | 460            | 2.85  | .10 |

## ONE WEEK AT 120° F. AND 65% R.H.

|                    | Fog   |       |       |       |
|--------------------|-------|-------|-------|-------|
|                    | Speed | Gamma | Speed | Gamma |
| Control.....       |       |       |       | .26   |
| I.....             |       |       |       | .95   |
| I plus phenol..... |       |       |       | .63   |

## Example 10

A gelatino-silver iodobromide emulsion digested with sulphur and gold sensitizing compounds was divided into

three parts. One part was treated with 45.5 grams of the poly-N-vinyl-2-pyrrolidone described in Example 1 per mole of silver halide. To a second part of the emulsion were added 45.5 grams of the polymer and 20 millimoles of 4,4'-n-butylidine-bis (2-t-butyl-5-methylphenol) per mole of silver halide. Neither of these additions was made to a third part of the emulsion.

Coating, exposure, development and aging were carried out as in Example 1.

## FRESH RESULTS

| Compound      | Amount per mole             | No. 2 exposure |       | No. 1 exposure |       | Fog | Covering power |
|---------------|-----------------------------|----------------|-------|----------------|-------|-----|----------------|
|               |                             | Speed          | Gamma | Speed          | Gamma |     |                |
| Control       | None                        | 800            | 3.11  | 390            | 2.49  | .06 | 25.5           |
| I             | 45.5 g.                     | 850            | 4.00  | 450            | 3.28  | .10 | 35.4           |
| I plus phenol | 45.5 g. (I), 20 mil-limoles | 800            | 4.05  | 400            | 3.42  | .08 | 32.5           |

ONE MONTH ROOM AGING

|                    | No. 2 exposure |       | No. 1 exposure |       | Fog |
|--------------------|----------------|-------|----------------|-------|-----|
|                    | Speed          | Gamma | Speed          | Gamma |     |
| Control.....       | 750            | 3.22  | 390            | 2.45  | .05 |
| I.....             | 800            | 3.55  | 440            | 2.93  | .14 |
| I plus phenol..... | 740            | 3.82  | 430            | 3.05  | .10 |

*Example 11*

A gelatino-silver iodobromide emulsion digested with sulphur and gold sensitizing compounds was divided into three parts. One part was treated with 45.5 grams of the poly-N-vinyl-2-pyrrolidone described in Example 1 per mole of silver halide. To a second part of the emulsion were added 45.5 grams of the polymer and 20 millimoles of 2,2'-methylene-bis (4-t-butyl-6-methylphenol) per mole of silver halide. Neither of these additions was made to a third part of the emulsion.

Coating, exposure, development and aging were carried out as in Example 1.

## FRESH RESULTS

| Compound      | Amount per mole             | No. 2 exposure |       | No. 1 exposure |       | Fog | Covering power |
|---------------|-----------------------------|----------------|-------|----------------|-------|-----|----------------|
|               |                             | Speed          | Gamma | Speed          | Gamma |     |                |
| Control       | None                        | 800            | 3.11  | 390            | 2.49  | .06 | 25.            |
| I             | 45.5 g.                     | 850            | 4.00  | 450            | 3.28  | .10 | 35.            |
| I plus phenol | 45.5 g. (I). 20 mil-limoles | 770            | 4.30  | 400            | 3.61  | .08 | 32.            |

ONE MONTH ROOM AGING

|                    | No. 2 exposure |       | No. 1 exposure |       | Fog |
|--------------------|----------------|-------|----------------|-------|-----|
|                    | Speed          | Gamma | Speed          | Gamma |     |
| Control.....       | 750            | 3.22  | 390            | 2.45  | .0  |
| I.....             | 800            | 3.55  | 440            | 2.93  | .1  |
| I plus phenol..... | 720            | 3.96  | 400            | 3.20  | .0  |

ONE WEEK AT 120° F. AND 65% R.H.

|                    | Fog |
|--------------------|-----|
| Control.....       | .2  |
| I.....             | .9  |
| I plus phenol..... | .5  |

As will be apparent from the above description, the invention is not limited to the use of the specific copolymers and homopolymers of the examples as various other such polymers can be used, e.g., poly-N-vinylcaprolac-

tam, poly-N-vinylvalerolactam and poly-N-vinyl-5-methyl-2-pyrrolidone and copolymers of two or more of the corresponding monomers. Also, copolymers of the latter with vinyl salicylate, vinyl acetate, vinyl alcohol, vinyl oxazolidone, methyl acrylate, acrylamide, methacrylamide, acrylonitrile, vinyl chloride, vinylidene chloride, and styrene containing at least 80% by weight of the poly-N-vinylactam. The N-vinyl-oxazolidone can be prepared by the method described in *J. Org. Chem.* 22, 849 (1957).

10 An advantage of this invention is that it provides a simple and effective way of improving the stability and aging characteristics of gelatino silver halide photographic emulsions containing substantial amounts of poly-N-vinylactams. It enables one to obtain the advantages  
15 of the covering power of such emulsions and overcomes their tendency to fog during normal or tropical storage conditions. The invention does not require expensive chemicals or involved procedures and can be carried out by the ordinary technician. Still further advantages will  
20 be apparent from the above.

What is claimed is:

What is claimed is:

1. A photographic silver halide emulsion comprising on a dry-weight basis 30% to 70% silver halide, 10% to 60% gelatin, 8% to 50% of an organic water-soluble addition polymer taken from the group consisting of homopolymers of at least one N-vinylactam containing 4 to 5 carbon atoms in the heterocyclic ring and copolymers of such an N-vinylactam with an ethylenically unsaturated compound taken from the group consisting of vinyl salicylate, vinyl acetate, vinyl oxazolidone, methyl acrylate, acrylamide, methacrylamide, acrylonitrile, vinyl chloride, vinylidene chloride and styrene containing at least 80% by weight of said N-vinylactam, and 5 to 50 millimoles per mole of silver halide of a phenol antifogging agent taken from the group consisting of (a) a hydrocarbon-substituted monohydric phenol of at least 10 carbon atoms having a hydrocarbon substituent in the para-position to the hydroxy group and 0 to 4 additional hydrocarbon substituents in the remainder of the benzene ring, said hydrocarbon substituents being the sole substituents in said phenol and being members taken from the group consisting of alkyl, aryl, aralkyl and cycloalkyl substituents, (b) hydrocarbon-substituted mononuclear monohydric phenols of at least 10 carbon atoms wherein the hydrocarbon substituents contains 4 to 12 carbon atoms and is in one of the positions ortho- and meta- to the hydroxyl group and other positions of the benzene ring are unsubstituted, (c) a compound of the general formula:



wherein Q is a member taken from the group consisting of a direct carbon-to-carbon linkage, —O—, —S—, —(CH<sub>2</sub>)<sub>n</sub>— where n is 1 to 4 and



where each of R and R<sub>1</sub> is alkyl of 1 to 18 carbon atoms,  
 65 and R' and R'' are each a member taken from the class  
 consisting of hydrogen, alkyl of 1 to 18 carbon atoms,  
 cycloalkyl and aryl, and (d) resorcinol.

2. An emulsion as defined in claim 1 wherein said silver halide is silver iodobromide.

70 3. An emulsion as defined in claim 1 wherein said

polymer is poly-N-vinyl-2-pyrrolidone.

References Cited in the file of this patent  
UNITED STATES PATENTS

|           |                |               |
|-----------|----------------|---------------|
| 2,495,918 | Bolton         | Jan. 31, 1950 |
| 2,553,506 | Mueller et al. | May 15, 1951  |
| 2,712,995 | Weyde          | July 12, 1955 |
| 2,732,300 | Thirtle et al. | Jan. 24, 1956 |
| 2,948,614 | Allen et al.   | Aug. 9, 1960  |
| 2,955,037 | Smith          | Oct. 4, 1960  |

|                                                                                |               |               |
|--------------------------------------------------------------------------------|---------------|---------------|
| 2,955,038                                                                      | Smith         | Oct. 4, 1960  |
| 2,965,487                                                                      | Smith         | Dec. 20, 1960 |
| FOREIGN PATENTS                                                                |               |               |
| 687,751                                                                        | Great Britain | Feb. 18, 1953 |
| OTHER REFERENCES                                                               |               |               |
| Mees: "The Theory of Photographic Process," page 679, The Macmillan Co., 1954. |               |               |